

# UNITED STATES PATENT OFFICE.

MAX DETHLEFFS, OF STUTTGART, GERMANY, ASSIGNOR TO CARL F. W. SCHNEEMANN,  
OF HANOVER, GERMANY.

## PROCESS FOR OBTAINING A MAT-SURFACE ON PRINTED MATTER WITH GLOSSY SURFACE.

1,057,624.

Specification of Letters Patent.

Patented Apr. 1, 1913.

No Drawing.

Application filed June 10, 1911. Serial No. 632,513.

*To all whom it may concern:*

Be it known that I, MAX DETHLEFFS, residing at Immenhoferstrasse 27, Stuttgart, Germany, printer, have invented a certain new and useful Process for Obtaining a Mat-Surface on Printed Matter with Glossy Surface, of which the following is a specification.

This invention relates to a process for removing the gloss from impressions, more particularly from colored illustrations, printed on glossy paper or cardboard with the customary printing colors, and to give such impressions a mat surface resembling that of an engravure.

The essential feature of the improved process according to my present invention consists in applying to the previously printed glossy impression, a paste of which the main constituents are soap and drying oils which are partially saponified by ammonia, along with an organic or inorganic substance adapted to produce a mat effect.

The coloring matter used in the printing need not be of special composition, any good printing color for illustrations being suitable, but to obtain the best results it is to be recommended that the coloring matter employed should contain slightly less drying agent than usual.

A paste of the following composition has proved very efficient, and is given by way of example:

|    |           |                         |
|----|-----------|-------------------------|
| 35 | 325 parts | Hanko or wood oil.      |
|    | 200 "     | boiled linseed oil.     |
|    | 150 "     | dry hydrate of alumina. |
|    | 50 "      | zinc borate (drier)     |
|    | 250 "     | white potassium soap.   |
| 40 | 25 "      | ammonia.                |

1,000 parts.

These ingredients are intimately mixed to

form a paste of thoroughly uniform activity, which in carrying out the process, is coated 45 or printed over the glossy surface of the paper or cardboard, the dry hydrate of alumina forming the filling material.

To overcome the odor of the wood-oil it is preferable to add a small amount of perfume to the mixture. The paste has the property of loosening the printing color to some extent and of removing its gloss, so that a soft, engravure like effect is obtained. The paste may obviously be colored or tinted 55 as desired.

My improved process is suitable for printing in more than one color.

Having now described my invention, what I claim as new and desire to secure by Letters Patent is:—

1. A process for obtaining a mat surface on printed matter with glossy surface, consisting in applying to the previously printed glossy impression a paste of which the main 65 constituents are soap and drying oils which are partially saponified along with a filling material thereby loosening the printing color to some extent and removing its gloss.

2. A process for obtaining a mat surface 70 on printed matter with glossy surface, consisting in applying to the previously printed glossy impression a paste of which the main constituents are soap and drying oils which are partially saponified along with a filling 75 material and a coloring material thereby loosening the printing color to some extent and removing its gloss.

In testimony whereof I have signed my name to this specification in the presence of 80 two subscribing witnesses.

MAX DETHLEFFS.

Witnesses:

ERNEST SCHNEEMANN,  
FRIDA KLAIBER.